

## UNITED STATES PATENT OFFICE

DAVID ALEXANDER WHYTE FAIRWEATHER, OF GRANGEMOUTH, AND JOHN THOMAS, OF KINGARTH, POLMONT, SCOTLAND, ASSIGNEES TO IMPERIAL CHEMICAL INDUSTRIES LTD., A CORPORATION OF GREAT BRITAIN

## DYE AND DYEING

No Drawing. Application filed December 9, 1930, Serial No. 501,160, and in Great Britain December 9, 1929.

This invention relates to dyes and dyeing and more particularly to the development of esters of vat dyestuffs and the like acid enolic ethereal salts of vat dyestuffs or quinones for example sulphuric esters, whether these esters are prepared from vat dye stuffs or from leuco bodies or from other appropriate starting materials.

The development of such esters by means of oxidizing agents such as ferric sulphate is known.

It is an object of the invention to provide improved or modified processes for the development of such esters.

We have observed that the development of esters of this type appears to be in part a reversible reaction, and our invention consists in a suitable adjustment of this reversible reaction so as to facilitate the development of the colour or to prevent over oxidation. We achieve this result, for example, in the case of development with ferric salts by the addition of a little ferrous salt or by the addition of salts of weak acids capable of forming double salts with the ferric salt present. In the case of development with copper salts, in which it is probable that the copper salt is converted into cuprous salt, acid and oxygen (the oxygen being utilized in developing the ester), we achieve this same result by reducing the concentration of acid originally present.

In developing dyeings of the esters of reduced vat dyestuffs using ferric sulphate we have found that the addition of ferrous sulphate is of great advantage, for instance, using ferric sulphate alone it is very easy to obtain over-oxidation, particularly with certain dyestuffs, for example, those belonging to the indanthrone class.

By the use of ferrous sulphate it is possible to easily avoid any over-oxidation. This result is very unexpected, since the addition of a reducing agent would not be expected to have any effect on the developing process.

One special advantage of this addition of ferrous sulphate is that it is possible to regulate the strength of the oxidizing agent with precision to suit any particular dyestuff by varying the relative proportions of ferric and

ferrous sulphate. The oxidation is preferably carried out in the presence of acid.

Instead of using ferric sulphate and ferrous sulphate, ferric chloride and ferrous chloride or other pairs of ferric and ferrous salts may be used.

It is possible that the beneficial effect of the ferrous salt is due to the fact that the reduction of a ferric to a ferrous salt is a reversible reaction.

Instead of using pairs of salts with the same acid, such as ferric sulphate and ferrous sulphate it is possible to use ferric and ferrous salts of different acids for instance, ferric chloride and ferrous sulphate. Using ferric sulphate and ferrous sulphate and acidulating, sulphuric acid forms a convenient acid. With ferric chloride and ferrous sulphate, hydrochloric acid forms a convenient acid. Salt may be added in addition.

It is possible to omit addition of a ferric salt altogether, and form it in situ, it being practicable, for example, to work with ferrous sulphate and sulphuric acid in the presence of air, but for large-scale operations development under these circumstances may not be sufficiently fast.

Another method of developing a ferric salt is to use a ferrous salt in conjunction with an oxidizing agent, for example, a nitrite or persulphate and in these cases a small quantity of the additional oxidizing agent will sometimes be found sufficient.

It is known to develop esters of reduced vat dyestuffs and similar substances by the use of copper salts in acid solutions.

One of the great advantages of the use of copper salts in this connection is the wide range of applicability of the copper salts and the fact that it is easy to carry out the oxidation without over-development.

The use of acid is common to nearly all methods of developing esters of reduced vat dyestuffs but we have discovered that reducing the concentration of acid in developing with copper salts increases instead of reduces the developing power; thus, a solution of cupric chloride is a stronger developing agent than a solution of cupric chloride containing hydrochloric acid. The actual strength of

the developing agent can therefore be varied and controlled by altering the strength of the acid.

This phenomenal result has the advantages that it is possible to eliminate or to reduce the concentration of the acid and also that development can be made to take place more rapidly. In carrying out this part of the invention cupric chloride may be used, or alternatively copper sulphate with the addition of sodium chloride.

The explanation of the phenomenon is probably to be found in the fact that the reduction of cupric salts, to give cuprous salts, acid, and oxygen, is a reversible reaction.

When using ferric salts as developing agents for the ester salts of reduced vat dyestuffs the addition of salts of weak acids which will form double salts with the ferric salts presents certain advantages.

As is known in using ferric salts, particularly with some dyestuffs which are easily over-oxidized, over-development is liable to take place.

The foregoing method however is of special use in avoiding over-oxidation, whilst the use of double salts obtained from ferric salts and salts of strong acids is not of the same advantage, since with these the liability to over-oxidation still exists.

The present invention, therefore, includes the use of double salts in the manner which is mentioned, preferably in the presence of a small quantity of acid.

The invention is further illustrated by the following examples in which the parts are parts by weight.

#### Example 1

Wool dyed with the sulphuric ester salt of indanthrone, for instance, 3 per cent of the ester salt calculated on the weight of the fibre, is developed in an aqueous bath containing 2 per cent hydrated ferrous sulphate, 1/2 per cent hydrated ferric sulphate and 1 per cent sulphuric acid. The bath is raised to 90° C. and the dyed wool is immersed in it for about 5 minutes. No super-oxidation occurs even if the development is carried on for over 10 minutes, and a pure bright blue shade results.

#### Example 2

In place of the ferric sulphate used in Example 1 in a bath otherwise of the same composition, an equivalent quantity of an oxidizing agent such as persulphate, bichromate, &c., may be added, these probably oxidizing part of the ferrous sulphate to the ferric state and so producing a bath of the same oxidizing power as in Example 1.

#### Example 3

Woolen cloth dyed with 4 per cent times its weight of the sulphuric ester salt of leuco

indigo is developed in the following bath:—

To a 1000 parts of an aqueous solution containing 2 per cent hydrated ferrous sulphate and 1 per cent sulphuric acid is added 1 part of sodium nitrite. The dyeing is immersed in the brown solution thus obtained and development is complete in about one hour in the cold. This time may be reduced to about ten minutes by warming the bath to 65° C.

#### Example 4

Cotton cloth is padded with a 2 per cent solution of the tetra-sulphuric ester of leuco indanthrone and dried.

The yellow dyeing so obtained is developed in the bath specified in Example 3 for 10 minutes at 80° C. Blue dyeings of exceptional brightness are thus produced, and the time of development and temperature may be varied within wide limits without super-oxidation to the yellow azine occurring.

If necessary 10 per cent of sodium chloride or sulphate may be added to the developing bath to prevent bleeding of the colour.

#### Example 5

Cotton cloth padded with a 2 per cent solution of the tetra-sulphuric ester salt of leuco indanthrone is developed in bath containing 2 per cent hydrated ferrous sulphate, 1/2 per cent hydrated ferric sulphate and 1/2 per cent sulphuric acid for 20 minutes at 50° C. The time and temperature may be considerably varied.

#### Example 6

In place of ferric sulphate in Examples 1 and 5 an equivalent quantity of ferric chloride may be used.

#### Example 7

Cotton cloth is dyed with the ester salt of leuco - Bb2 : Bz2' - dimethoxydibenzanthrone (caledon jade green) and the orange brown dyeing is immersed either in the bath specified in Example 3 or that of Example 5 in the cold for a few minutes.

#### Example 8

Wool dyed as in Example 1 is developed in a bath containing 40 parts of a 10 per cent solution of ferric chloride, 360 parts of a 2 per cent solution of ammonium oxalate crystals, 5 parts of concentrated hydrochloric acid, and 160 parts of water, for 4 minutes at 90° C.

#### Example 9

Cotton cloth padded as in Example 4 is immersed at 90° C. in a 2 per cent solution of crystalline cupric sulphate in water. Development proceeds rapidly and the dyeing may be lifted and rinsed in about 5 minutes.

*Example 10*

Wool dyed as in Example 1, is developed in an aqueous bath containing 2 per cent ferric ammonium citrate and 0.2 per cent sulphuric acid, for 30 minutes at 90° C.

*Example 11*

The added substances in the developing bath in the previous example may be replaced by the following: Ferric ammonium tartrate 2 per cent, neutral sodium tartrate, 2 per cent, and hydrochloric acid liquor, 3 per cent. Development is complete in 5 minutes at 90° C. when a bright blue dyeing is obtained.

*Example 12*

The proportions of the constituents of a developer containing ferrous sulphate may be considerably varied without appreciably altering the shade produced in the case of a dyeing with an indanthrene ester. A smaller quantity of ferrous sulphate than in the previous examples is satisfactory when the fabric is of wool, employing the following bath containing 2 parts hydrated ferric sulphate, 5 parts hydrated ferrous sulphate and 5 parts sulphuric acid in 1000 parts of water. Development may be carried on at 85° C. for 15-30 minutes.

*Example 13*

In place of ferrous sulphate in any of the previous examples, ferrous ammonium sulphate in proportionately larger quantity may be employed. The development is somewhat retarded and a slightly longer time in the bath is usually necessary for the production of the correct shade.

*General*

The invention is not limited to sulphuric esters.

The invention includes development of the dyestuff in substance. It includes colouring generally, for instance, dyeing as well as printing and padding.

As many apparently widely different embodiments of this invention may be made without departing from the spirit and scope thereof, it is to be understood that we do not limit ourselves to the specific embodiments thereof except as defined in the appended patent claims.

We claim:

1. Process for the development of enolic leuco-ester salts of dyestuffs in the presence of a ferric salt characterized by the addition of an agent capable of influencing the reversible reaction which the ferric salt undergoes during the development, said agent being a salt of the class consisting of ferrous salts and salts of weak acids capable of forming double salts with said ferric salts.
2. Process according to claim 1 in which the added agent is a ferrous salt.

3. Process according to claim 1 in which the added agent is a salt of a weak acid which salt is capable of forming a double salt with the ferric salt.

4. Process according to claim 1 in which the development occurs in the presence of ferric sulphate and the added agent is ferrous sulphate.

5. Process according to claim 1 in which the added agent is an ammonium salt of a weak acid.

6. Process according to claim 1 in which the added agent is ammonium oxalate.

7. Process according to claim 1 in which there is present, in addition to the ferric salt, another developing agent.

8. Process according to claim 1 in which there is present, in addition to the ferric salt, a substance capable of generating nitrous acid.

9. Process according to claim 1 in which the ferric salt is generated in situ by oxidation of a ferrous salt.

10. Process according to claim 1 in which part of the ferric salt is generated in situ by oxidation of a ferrous salt.

11. Process according to claim 1 in which, in addition to a ferric salt as developer and a ferrous salt as agent for influencing the reversible reaction, there is also present another oxidizing agent.

12. Process according to claim 1 in which a small quantity of acid is also present.

13. Process for the development of enolic leuco-ester salts of dyestuffs in the presence of ferric sulphate, ferrous sulphate, and sulphuric acid.

14. Process for the development of enolic leuco-ester salts of dyestuffs in the presence of a ferric salt, characterized by the employment of the ferric salt in the form of a double ferric salt of a weak acid.

15. Process according to claim 14 in which the double ferric salt used is a ferric ammonium salt of an organic carboxylic acid.

16. Process according to claim 14 in which a small quantity of acid is also present.

17. A process of developing enolic/leuco-ester salts of dyestuffs which comprises immersing a fabric impregnated with said ester salts, in a developing bath comprising an oxidizing agent and a ferrous salt and effecting the development of said dyestuffs.

18. The process of claim 17 in which said oxidizing agent is a ferric salt.

In testimony whereof we affix our signatures.

DAVID ALEXANDER WHYTE FAIRWEATHER.  
JOHN THOMAS.

125

130

CERTIFICATE OF CORRECTION.

Patent No. 1,886,947.

November 8, 1932.

DAVID ALEXANDER WHYTE FAIRWEATHER ET AL.

It is hereby certified that error appears in the printed specification of the above numbered patent requiring correction as follows: Page 2, line 95, after "in" insert the words "an aqueous"; and line 109, for the syllable "Bb2" read 'Bz2'; and that the said Letters Patent should be read with these corrections therein that the same may conform to the record of the case in the Patent Office.

Signed and sealed this 27th day of December A. D. 1932.

(Seal)

M. J. Moore,  
Acting Commissioner of Patents.